

March 19, 1963

A. W. HARRIS

3,082,119

METHOD OF AND APPARATUS FOR HOT-DIP COATING STRANDS

Filed Feb. 24, 1960

2 Sheets-Sheet 1



INVENTOR  
ARCH W. HARRIS  
By Donald G. Dalton  
Attorney

March 19, 1963

A. W. HARRIS

3,082,119

METHOD OF AND APPARATUS FOR HOT-DIP COATING STRANDS

Filed Feb. 24, 1960

2 Sheets-Sheet 2



FIG. 4



INVENTOR  
ARCH W. HARRIS  
By Donald G. Dalton  
Attorney

## 1

3,082,119

**METHOD OF AND APPARATUS FOR HOT-DIP COATING STRANDS**

Arch W. Harris, Warrensville Township, Cuyahoga County, Ohio, assignor to United States Steel Corporation, a corporation of New Jersey

Filed Feb. 24, 1960, Ser. No. 10,639

6 Claims. (Cl. 117—114)

This invention relates to an improved method and apparatus for hot-dip coating a continuous metallic strand with a metal or alloy having a substantially lower melting point than the metal or alloy of the strand and more particularly to an improved method for the continuous hot-dip coating of a steel strand with a molten metal, such as aluminum, which does not readily wet steel.

Conventional processes of hot-dip coating are of two general varieties. The first is characterized by passing the cleaned base metal through a flux and then into a molten bath of the coating metal. In the second, the cleaned metal is heated in a reducing atmosphere and passed into the molten coating metal while still under the protection of the atmosphere. The aim in both instances is to bring clean metallic surfaces into contact and thus achieve a complete wetting of the base metal with the molten coating metal. Complete wetting is essential to avoid "black-spots," (uncoated areas). It is well recognized that the use of flux, either liquid or gaseous, for this purpose presents several disadvantages. Moreover, this critical objective is not attained by either conventional procedure when applied in the coating of a continuously moving strand except at rather low rates of strand movement. In the case of aluminum coated steel wire, black-spots are not completely eliminated even at impractically low strand speeds.

Accordingly it is an object of the present invention to provide an improved continuous hot-dip coating process wherein smooth coatings free of even minute uncoated areas can be produced at high speed without use of fluxes or preheating in a reducing atmosphere.

Another disadvantage of prior art practices has been the inability to produce a perfectly aluminum coated strand having high tensile strength. This derives from the fact that the coating bath must be maintained at a temperature of 1100 to 1300 F. depending upon the purity of aluminum used and the steel brought to this temperature by the bath itself or by preheating. Thus in conventional practices because of the relatively slow rates of strand travel, the steel is substantially annealed, and the desired effects of prior cold working or heat treatment to raise tensile properties of the steel are largely lost. Similar difficulties, but to a somewhat lesser degree are encountered in continuous hot galvanizing and tinning operations.

Accordingly another object of the invention is the provision of hot-dip coating process in which time at coating temperature is so short that physical properties of the base metal are not substantially reduced thereby; a particular object being production of hot-dip aluminum coated steel strands having tensile strength in excess of 200,000 p.s.i.

Another problem encountered in adapting conventional procedures of hot-dip aluminum coating of steel strands has been the control of thickness of the alloy layer produced during the passage of the strand through the molten coating bath. The development of some intermetallic compounds between the base and coating metals is beneficial, increasing adherence, improving soldering characteristics and the like. Excessive alloy however is detrimental, consequently control of alloy formation has been the subject of intensive investigation. Since maximum speed of travel in conventional hot-dip procedures is fixed

## 2

by other considerations, the conventional solution to alloy control has been to alloy the coating bath with a metal which tends to suppress alloy formation. While such practices have been successful to a considerable degree, they introduce certain undesirable limitations, for example, the use of a few percent of silicon in the aluminum bath reduces the alloy formation but at the same time adversely affects other characteristics of the coating itself.

Accordingly, it is a further object of the invention to provide an improved process which permits the use of unalloyed coating baths.

Other objects will appear as the description proceeds.

Heretofore control of black-spots to even a reasonable degree in the hot-dip aluminum coating of steel has required limiting strand speed to a maximum of about 40 feet per minute; the maximum varying somewhat with the dimensions of the strand being coated. Even at such slow speeds some black-spots or holidays are caused by gas evolution from the steel base through the molten coating just before or just after emergence from the coating bath. I have found this speed limitation is removed and black-spots and the like, completely eliminated by imparting, in combination with certain other practices hereafter described, vibratory forces of a particular nature to the strand as it enters the aluminum bath. Moreover, I have found that these practices make an unexpectedly large reduction in the time of immersion and that the strand leaving the coating bath not only carries a complete coating but little or no alloy is formed thereon during its passage through the bath.

I am aware that the use of vibration to promote wettability in soldering operations and the like has been proposed. However, such earlier proposals have in general been concerned with ultrasonic vibrations and have never been successfully applied in the continuous coating operations outlined above. I have found that success in the latter operations requires strict adherence to the following principles:

Firstly, the vibratory force must be applied in such manner as to develop a transient, random vibration in the strand, such being characterized by innumerable frequencies in excess of 80 cycles per second and an overall acceleration in excess of 20 g. Secondly, the vibratory force must be applied to the strand as near its entry into the pool as is practical; the vibrations or vibratory energy imparted to the strand must be substantially dissipated or damped out before the strand is discharged from the coating pool into the atmosphere and the strand must be moved at substantially no tension. The foregoing conditions are essential to avoiding the development of standing waves in the exiting strand which cause rough, uneven coating and even extensive uncoated areas.

The term "substantially no tension" as used herein is understood to mean not substantially more tension than is required to move the strand through the apparatus and excludes the application of appreciable back tension.

The required transient, random type of vibrations are produced in the strand by applying shock impulses at regular intervals while restraining movement of the strand in the direction of the blow. The aim is to produce slight random movement of the strand rather than movement of a particular amplitude in a particular plane. Accordingly, results are not associated with development in the strand of motion having a particular frequency and level of acceleration but rather with the development of an extremely complex motion in which substantially all frequencies over a relatively wide range falling within the audible frequency band are present at about the same level of acceleration. I have not, for example, been able to produce coatings at high speeds completely free of black-spots by inducing a pure sinusoidal vibration in the strand. A minimum of 40 to 60 shock impulses per

second is required; while rates of several thousand impulses per second can be used. Intermediate rates ranging from 100 to 1000 impulses per second, however, afford an ample operating range for all conditions normally encountered; the optimum rate within this range depending on the mass of strand, the degree with which movement of the strand in the direction of impact is limited, and to some extent on the design of the vibrator itself. The lowest frequency developing in the strand should be of the order of 80 c.p.s. but may be as high as about 400 c.p.s. without adverse effect. Absence of frequencies below about 300 c.p.s. requires higher overall accelerations which while not detrimental is wasteful of vibrating power. The highest frequency developing in the strand may be in excess of 16,000 c.p.s. however the absence of frequencies over about 3000 c.p.s. is not detrimental. The intensity of the induced vibrations is important and is conveniently defined in terms of acceleration as multiples of  $g$ , the acceleration of gravity, 32.172 ft./sec./sec. In this regard, the value of acceleration associated with the full range of frequencies present in the motion, i.e., the overall acceleration, is the determining factor. The required motion being both transient and random, the acceleration associated with any particular component (frequency) thereof may vary considerably from moment to moment; the overall acceleration however, remains relatively constant and must be maintained at at least 20  $g$  for satisfactory coating results. Overall accelerations as high as 5000  $g$  have produced good results, but I prefer to use the lowest acceleration commensurate with good results since more efficient use of vibrating power with least wear of the vibrator is achieved. The important point in this regard is that the vibrations and vibratory energy imparted to the strand must be substantially above that which would be absorbed or dissipated by the passage of the strand through the coating bath. A minimum acceleration of 20  $g$  achieves this result. Optimum value of acceleration varies with the material, temper, shape and dimensions of the strand, the design of the imparting vibrator and its associated motion limiting device and thus must be determined experimentally for each installation. The presence of discrete peaks in the frequency-acceleration curve are not detrimental, although extremely high level peaks toward the lower end of the frequency range may, under some conditions, contribute to the formation of standing waves in the exciting strand, which condition must be avoided if smooth, black-spot free coatings are to be produced.

Control of motion in the strand is conveniently accomplished by regulating the rate of application of the shock impulses. Other factors being equal, the range of frequencies developing in the strand can be shifted upwardly and, more importantly, the overall acceleration associated therewith can be increased by increasing the impact rate. The frequency range and acceleration can also be altered by increasing the restriction of strand movement in the direction of impulse application. Restricting strand movement increases the energy imparted per blow and contributes to randomness of the motion achieved, for example, using an impact rate of 300 impulses per second against a restricted No. 10 gage low carbon steel wire moving at 75 f.p.m. induced vibrations having an overall acceleration of 1000  $g$  and produced an excellent aluminum coating; removing the restriction however altered the characteristics of the motion in the wire sufficiently to adversely affect the coating and required increasing the impact rate to 900 impulses per second to restore coating quality. Accordingly, it is preferable in practicing my invention to use a fixed degree of restriction at the imparting vibrator and adjust the impact rate if required.

Characteristics of the vibratory motion required in the present method were determined using an Endevco accelerometer and amplifier, a tape recorder, and a Brüel & Kjaer frequency analyzer and graphic level recorder.

A tape recording of the amplified output voltage of the accelerometer was made while the vibration pick-up of the instrument was held manually against the vibrating strand. A loop of the tape was then played back continuously on the tape recorder and the electrical voltage produced was fed through the analyzer into the graphic level recorder to produce a graph of vibration level as a function of frequency. The overall acceleration was computed from the graphed data.

In addition to greatly promoting wettability, induced vibratory motions of the character described, greatly increases the rate of heat transfer from the coating bath to the strand. The magnitude of the latter effect is such that time of immersion in the bath must be limited to a maximum of about 8 seconds if the benefits of the invention are to be obtained. Immersion time is a function of length of immersion and speed of strand travel through the bath and is fixed in design of the coating pot and rigging. A minimum immersion of about 0.5 second must be provided to produce satisfactory coating. Where minimum alteration of physical properties of the base metal is required, the immersion time should be as short as possible and preferably not more than about 3 seconds. The maximum in this regard varies somewhat with mass of the strand and bath temperature.

A preferred arrangement of processing steps and apparatus suitable for the practices of my invention is shown in the attached drawing, in which:

FIGURE 1 is a schematic side elevation, partly in section of a coating line embodying the principles of my invention;

FIGURE 2 is an enlarged longitudinal section of the coating pot of FIGURE 1;

FIGURE 3 is a partial end elevation of the coating pot;

FIGURE 4 is a plan of the vibration imparting mechanism;

FIGURE 5 is a sectional view taken along plane IV—IV of FIGURE 4;

FIGURE 6 is a side elevation of the hold-down mechanism;

FIGURES 7 and 8 are respectively, a front elevation and a plan view of a gas wipe particularly adapted to the practices of my invention; and

FIGURE 9 is a sectional view thereof taken along the plane IX-IX of FIGURE 8.

With particular reference to the drawing, the numeral 2 designates a coil of strand or wire S disposed on a pay-off reel 4 which is power driven and provided with conventional controls, not shown, for automatically regulating the speed thereof. Located at the other end of the line is a power-driven take-up reel or recoiler 40 also provided with conventional controls, not shown, for automatic speed regulation. Reels 4 and 40 are operated to feed and gather strand S at the same lineal rate so that the strand will be moved through the apparatus at substantially no tension. From the pay-off reel, the strand S may be fed through cleaning tank 6, preferably a tank of molten caustic and then through a water rinse 8. Alternately or sequentially the strand may be conducted through a tank 10 containing a dilute aqueous sulphuric or hydrochloric cleaning solution followed by a water rinse 12. Cleaning arrangement shown is particularly adapted to the removal of the lubricants and drawing compounds conventionally used in the cold drawing of wire. The molten caustic breaks down the drawing lubricants to a readily removable form and complete neutralization and cleansing is effected by the acid bath. Methods better adapted to other materials can, of course, be substituted. Preferably the strand is next conducted through a hot water rinse tank 14 to further rinse the strand, expel as much adsorbed gas as possible, and promote drying thereof. Drying is substantially completed by a hot-air or similar drier 16, after which the strand is passed into contact with a rotary impact-imparting mechanism V for inducing vibratory motion of the re-

quired character in the strand. An adjustable, resiliently mounted hold-down sheave 18 located just ahead of the mechanism V maintains the strand in suitable contact therewith to restrict strand movement in the direction of application of impact; the amount of such restriction being regulatable by adjustment of spring pressure on the sheave. From vibrator V the strand passes through an elongated tube 22 having one end submerged in a bath 20 of molten coating metal. A gas inlet 24 is provided adjacent the lower end of the tube and a nonoxidizing or reducing gas is continuously introduced to maintain a nonoxidizing atmosphere in contact with the bath surface at the point of entry of the strand. If the gas is combustible, it may be burned at the upper end of the tube as it exits therefrom. Vibratory motion induced in strand S rapidly dissipates any absorbed gas or water films from the strand and disrupts any oxide films formed on the bath surface, however, exceptionally heavy top dross is produced; accordingly, the steps for drying the strand and maintaining the bath surface free of oxide while not essential in the present method to the production of a quality aluminum coating, are included for economic reasons. The flow of gas through tube 22 carries away the gases and any water vapor evolved from the strand by the imparted vibration and maintains the surface of the coating metal at the point of strand entry completely free of oxide, accomplishing this objective without the formation of any deleterious side reaction products. In coating with zinc or tin, drying of the strand is, of course, a necessary safety measure. The strand is submerged in the coating metal by a sinker 26, passing therefrom in a substantially vertical pass-line to a deflector roll 34 located a sufficient distance above the bath to avoid contacting the strand prior to complete solidification of the coating thereon. Cooling means 35 arranged to direct a blast of cool air or atomized water against the strand to arrest alloy formation, may be positioned below sheave 34. Means 35 should be supported in an adjustable manner to be positionable in the pass as may be required. The coated strand leaves the bath through a specially constructed gas wipe 30, partially submerged in the molten coating metal. Wipe 30, shown in detail in FIGURES 7, 8, and 9, comprises an open-bottom, box-like chamber 30A having in the top thereof, an opening 31 for the passage of the coated strand and a gas inlet 32. A combustible gas, e.g. natural gas, is introduced at inlet 32 and burned at opening 31. The latter should be restricted to a size permitting a free flow of the gas completely around the exiting strand but preventing back-flow of air into the chamber. The burning gas promotes flow-back of excess coating metal and maintains the bath surface free of oxides and dross at the point of strand exit to insure bright, uniform coatings. Extending the width of chamber 30A several inches above the bottom thereof and disposed below opening 31 so as to contact a strand exiting therethrough is a rod 28 of "Alundum" or like material supported at one end by the blind recess in boss 27A and by the threaded opening in boss 27B at the other, threaded plug 27C serving to clamp the rod in this position. Rod 28 is preferably grooved to prevent strand S from rubbing the side walls of opening 31. Projecting from one side of chamber 30A and aligned to permit observation of the contact of strand S and bar 28 is a sight tube 29, the end of which is closed to the atmosphere by a suitable glass disc 29A and clamping ring 29B. Support arm 30B welded or otherwise attached to the back of chamber 30A, is slidably disposed in a clamp 33 which in turn is slidably attached to vertical standards 25 carried by the back wall 20A of the coating pot.

As previously mentioned, the present invention contemplates prevention of standing waves in the strand leaving the coating pot by maintaining the strand substantially untensioned and dissipating a substantial portion of the energy imparted by vibrator V before discharging the coated strand into the atmosphere. The

latter is accomplished by positioning wipe 30 so that bar 28 bears against strand S at a point 1½ to 3 inches above the surface of the molten coating metal to deflect the strand from the position it would, by reason of its substantially untensioned condition, otherwise normally assume in passing from sinker 26 to sheave 34. The degree of deflection must be such as will develop sufficient pressure to maintain a positive contact of strand and bar at all times, but insufficient to remove the coating at the point of contact.

Since for any given deflection, the pressure of contact depends upon the resilience of the strand which in turn varies with such factors as strand composition, its cross-sectional dimensions and prior treatments affecting its mechanical properties, the position of wipe 30 must be adjusted for different strands. It is impossible to assign numerical limits of either deflection or pressure, accordingly, necessary adjustments must be made by observation of results.

Location of contact bar 28 is of critical importance to the practical achievement of the results of my invention. Complete submersion favors dissipation of the vibratory energy from the strand and does so without damage to the coating. A completely submerged bar, however, behaves erratically; such bars frequently disintegrate in exceedingly short times. Moreover, adjustment of a submerged bar is very difficult and time consuming. On the other hand, rough, oxidized streaks and other coating defects resulting from contacting the molten coating can not be tolerated. I have found the foregoing difficulties are completely avoided and the required dissipation of vibratory energy achieved only if the contact is made within the gas wipe a few inches above the bath surface. Due to the upward drag of molten metal by the rapidly moving strand, the coating at this location is abnormally thick, is fully molten and is protected against oxidation by the atmosphere of the wipe. Under these conditions the disturbance of the coating by the squeegeeing action of the contact bar has no permanent effect and the coating produced is uniform and free of oxide streaks. For effective dampening, however, contact must be made with in 1½ and 3 inches of the bath surface, depending somewhat on the speed of travel, size, and mechanical properties of the strand. The bar is easily adjusted since contact can be observed through the sight tube 29.

From sheave 34 the coated strand may be conveyed by suitable arrangement of rolls or sheaves, through conventional means indicated at 36 and 38 to further cool treat, or lubricate the product as desired. Thereafter the strand is wound on take-up reel 40 previously described. Since it is essential to the purposes of my invention that the strand does not become taut during its passage through the equipment, care must be taken in design to minimize friction at, as well as the number of conveying rolls or sheaves. Straight-through-type treating tanks should be used wherever possible.

A preferred embodiment of the vibrator V is shown in FIGURES 4 and 5 of the drawing. It is comprised of a variable speed motor 50 connected to a pair of opposed discs 52. Disposed between the discs are a plurality of equally spaced pins or bars 54 spaced inwardly a slight distance from the periphery of the discs as shown in FIGURE 5. The assembly is supported on a plate 55 from the forward wall of coating pot 20 with the top edge of the discs 52 projecting above the normal pass line of the strand. Thus, the strand rides loosely between the discs and is subjected to an impact by each pin as the discs rotate. Hold-down sheave 18 positioned to ride the surface of the strand a slight distance ahead of disc 52 is carried by a bearing bracket 58 which is fitted to slide freely on a pair of support rods 60. A spring 62 is positioned between the bracket 58 and a retainer bar 64; the latter being adjustably secured to supports 66. Thus, sheave 18 resiliently urges the strand into contact with the pins and resiliently restricts the movement of

the strand in the direction of the impacts applied by the pins. Spring pressure determines the amount of restriction and is regulatable by adjusting the position of the retainer bar 64. Lateral displacement of the strand by the impacts is prevented by the projecting edges of discs 52. Conventional means (not shown), for controlling the speed of the motor 50 are provided so that the impact rate may be regulated. Direction of rotation of motor 50 is selected to drive discs 52 in the direction of strand travel to aid strand movement through the coating bath and thus minimize tension build-up. Thus, the described arrangement is particularly suited to the purposes of the present invention.

The following specific examples serve to illustrate the practices and results of the invention.

*Example A*

Cold drawn, high-carbon steel wire, size 0.103", grade SAE C-1085 having a tensile strength in excess of 200,000 p.s.i., was hot-dip coated with aluminum containing 3% silicon at a speed of 130 f.p.m. to provide a defect free coating without affecting the tensile properties of the steel by the following sequence of treatment:

The wire was continuously fed from a pay-off reel 4 and passed successively through molten sodium hydroxide, maintained at between 800 and 950° F. in tank 6, water rinse 8, a cold dilute muriatic acid bath 10 and a cold water rinse 12 to remove the drawing lubricant and any foreign material from the surface thereof. The cleaned wire was dried by passing it through hot water tank 14 and hot-air drier 16. Hold-down sheave 18 was adjusted to provide a medium level of resilient restriction and the vibrator V, which consisted of ten (10)  $\frac{3}{8}$ " diameter pins 54, equally spaced about a  $5\frac{1}{8}$ " diameter circle on discs 52, was rotated to impart 360 impacts per second to the wire. These particular conditions induced vibrations in the wire having frequencies continuously distributed over the frequency range 80 to 10,000 c.p.s. at an overall acceleration of 1200 g. The wire was introduced into the coating pot through tube 22 in which a small flow of natural gas was maintained through inlet 24, the gas being allowed to burn at the upper end of the tube. The bath was maintained at about 1200 F. and the length of wire immersion therein was about 4 feet, thus, provided an immersion time, at 130 f.p.m., of 1.85 seconds. After passing around sinker 26 the wire left the bath through gas wipe 30 wherein a small flow of natural gas was maintained through inlet 32 and allowed to burn around the strand at the opening 31. With the strand moving at speed (130 f.p.m.) the position of wipe 30 was adjusted to bring bar 28 into a uniform and positive contact with the wire at a point about  $1\frac{1}{2}$  inches above the bath's surface with a pressure just short of that which will cause a dry-streak or other damage in the coating. The wire was allowed to cool naturally to the solidification temperature of the coating in its upward passage to sheave 34. Temperature of the wire was further reduced by passing through warm water in tank 36, a film of oil applied in tank 38 and the coated wire recoiled by take-up reel 40. A clear, bright aluminum coating amounting to 0.36 oz. per square foot of wire surface was obtained. The coating was completely free of black-spots and could be formed into the standard "wire button" test without cracking or peeling. The alloy layer formed was uniform and slightly less than normal. Tensile tests of the wire showed substantially no change in the physical properties of the base metal.

*Example B*

Materials and conditions were the same as in Example A except that the use of the hot water rinse 14, the drier 16 and the bath entry tube 22 was eliminated. Insofar as product was concerned, results were the same as in A but, a large amount of top dross was produced at the entry end of the coating pot. While the dross did not

interfere with coating, it represents a substantial loss of coating metal.

*Example C*

Cold drawn wire, size 0.103", grade SAE C-1060 was coated using the same sequence as Example B except that acid cleaning 10 was also eliminated, the vibrator was operated to impart 450 impacts per second and the speed of the line reduced to 100 f.p.m. At this speed a coating of 0.295 oz. per square foot was produced. Overall acceleration of motion in the wire was 1000 g, immersion time in bath was 2.4 seconds. Coating was bright and completely free of black-spots, although the wire entering the coating pot carried a visible brown film.

*Example D*

The wire of Example C was coated using an impact rate of 175 impacts per second at a speed of 136 f.p.m. The overall acceleration of the vibratory motion imparted was about 400 g and immersion time in the bath was about 1.75 seconds. Again, clear, bright, black-spot free coatings of unusually high adherence were achieved.

*Example E*

Low carbon steel wire, size 0.0625, was coated using the sequences utilized in Example A. In this instance a vibrator consisting of sixteen (16)  $\frac{3}{8}$ " diameter pins equally spaced about a  $5\frac{1}{8}$ " diameter circle on discs 52 was rotated to impart about 600 impacts per second and the line operated at 120 f.p.m. Hold-down sheave 18 was adjusted to provide light pressure and three levels of overall acceleration (25, 60 and 100 g) in the motion induced in the wire. Time in the coating bath was 2.0 seconds. In all instances bright, clear, black-spot free coatings were produced.

*Example F*

Low carbon steel wire, size 0.135 inch was coated using the sequence outlined in Example A at 75 f.p.m. using a vibrator consisting of twelve (12)  $\frac{3}{8}$ " diameter pins equally spaced about a  $5\frac{1}{8}$ " circle on discs 52. Hold-down sheave 18 was adjusted to apply a medium restrictive pressure. The vibrator was rotated to apply impact rates varied 200 to 800 per second, inducing random transient motion in the wire at levels varying from 2000 to 2750 g. Immersion time was 3.2 seconds. Exceptional coatings were obtained over the entire range.

In general wires as small as 0.04" in diameter and as large as 0.238" have been coated successfully and all advantages of the present method achieved. Aluminum coatings amounting to 0.50 oz. per square foot have been applied to 0.080" size wire at 200 f.p.m.; also to 0.148 size wire at 150 and 220 f.p.m. In the case of large diameter wire, it has proven advantageous to use a rotating sinker and remove the wire from the bath at an angle rather than in a vertical pass; this reduces dragging at the sinker and aids in avoiding deleterious standing waves in the exit pass.

Speeds up to 250 f.p.m. (about six times the maximum speed possible heretofore), have been used. Operations at high speed permit reduction of the immersion time to less than 1 second. The latter, coupled with the fact that vibrating in the manner described greatly increases the rate of heat transfer, affords a degree of control of alloy formation not heretofore available. This may be illustrated by the fact that the coated wire of Example A can be produced substantially free of alloy layer by quenching the coated strand as it emerges through the gas wire by passing it through the cooling device 35 wherein it is sprayed with steam, atomized water or simply with a blast of cold air. This result is obtained even with a bath of substantially pure aluminum maintained at a temperature of about 1235 F. By regulating the position of cooler 35 in relation to the speed of travel of the strand, the optimum amount of alloy layer consistent with good adhesion, brightness of coating and other desired characteristics can be produced.

As used in the foregoing description, the term "strand" includes single continuous lengths of metallic strip or wire as well as a plurality of lengths twisted or otherwise grouped together.

This application is a continuation-in-part of my co-pending application Serial No. 743,616, filed June 23, 1958, now abandoned.

While the foregoing examples have illustrated application of my invention to the aluminum coating of steel, it is not limited thereto but can be applied with advantage in the continuous hot-dip galvanizing and tinning of steel and other basis metals.

I claim:

1. A method of producing cold drawn aluminum coated steel wire having a high tensile strength characterized by freedom from black spots from cleaned, cold drawn wire comprising continuously advancing the cleaned wire in a substantially untensioned condition through a flux-free bath consisting essentially of molten aluminum at a speed in excess of 40 feet per minute and with an immersion time of not more than about 3 seconds, applying at least 40 shock type impulses per second to the wire adjacent the entry portion of the bath while restricting movement of the wire in the direction of application of the shock type impulses adjacent the point of application thereof to produce transient random vibrations in the strand characterized by the presence of innumerable frequencies in excess of about 80 c.p.s. and an overall acceleration value in excess of 20 g whereby the surface of the wire is continuously wetted to form an uninterrupted molten sleeve of coating metal thereon, said vibrations having sufficient intensity to dislodge the coating metal from the wire as it emerges from the bath if not damped, the shock type impulses being applied to the wire in the direction of travel thereof to maintain the wire in said substantially untensioned condition, positively dampening the vibration of said substantially untensioned coated wire before it contacts the air to prevent the molten coating metal being dislodged therefrom, withdrawing said wire from the bath in an upward direction and quickly quenching the molten coating metal to minimize the alloy layer formation before changing the direction of movement of the coated wire.

2. A method of producing cold drawn aluminum coated steel wire having a tensile strength in excess of 200,000 p.s.i. characterized by freedom from black spots comprising cleaning the cold drawn wire to remove the cold drawing lubricants therefrom, continuously advancing the cleaned wire in a substantially untensioned condition through a flux-free bath consisting essentially of molten aluminum with an immersion time of not more than about 3 seconds, applying at least 40 shock type impulses per second to the wire adjacent the entry portion of the bath while resiliently restricting movement of the strand in the direction of application of the shock type impulses adjacent the point of application thereof to produce transient random vibrations in the strand characterized by the presence of innumerable frequencies in the range of about 80 to 10,000 c.p.s. and an overall acceleration value in the range of 100 to 1000 g whereby the surface of the wire is continuously wetted to form an uninterrupted molten sleeve of coating metal thereon, said vibrations having sufficient intensity to dislodge the coating metal from the wire as it emerges from the bath if not damped, withdrawing said substantially untensioned wire from the bath in vertical direction through a nonoxidizing atmosphere, positively dampening the vibration of said wire sufficiently as it leaves the bath and while in said nonoxidizing atmosphere to prevent the molten coating metal being dislodged therefrom and continuing the vertical travel of the wire for a sufficient distance to permit the molten metal to freeze with a smooth surface before changing the direction of movement of the coated wire.

3. A method of producing aluminum coated steel wire having good physical properties characterized by freedom from black spots from cleaned, cold drawn steel wire comprising continuously advancing the cleaned wire in a substantially untensioned condition through a substantially molten aluminum flux-free coating bath at a speed in excess of 40 feet per minute and with an immersion time of not more than about 8 seconds, applying at least 40 shock type impulses per second to the wire adjacent the entry portion of the bath while restricting movement of the wire in the direction of application of the shock type impulses adjacent the point of application thereof to produce transient random vibrations in the strand characterized by the presence of innumerable frequencies in excess of about 80 c.p.s. and an overall acceleration value in excess of 20 g whereby the surface of the wire is continuously wetted to form an uninterrupted molten sleeve of coating metal thereon, said vibrations having sufficient intensity to dislodge the coating metal from the wire as it emerges from the bath if not damped, positively dampening the vibrations of said substantially untensioned coated wire before it contacts the air to prevent the molten coating metal from being dislodged therefrom, withdrawing said wire from the bath in an upward direction and continuing the upward travel of the wire for sufficient distance to permit the coating metal to freeze with a smooth surface before changing the direction of movement of the coated wire.

4. Apparatus for continuously hot-dip coating strand comprising means for continuously advancing strand through a bath of molten coating metal, vibrating means at the entry end of the bath for imparting at least 40 shock type impulses per second to the strand and produce random, transient vibrations in the strand traveling through the molten coating metal characterized by the presence of innumerable frequencies in excess of about 80 c.p.s. and an overall acceleration value in excess of 20 g, positive vibration dissipating means at the exit end of the bath adapted to contact said strand prior to its discharge into the air, and means adjacent the vibrating means for resiliently restricting movement of the strand in the direction of application of the shock type impulses.

5. Apparatus for continuously hot-dip coating strand comprising means for continuously advancing strand through a bath of molten coating metal, rotary vibrating means at the entry end of the bath for imparting at least 40 shock type impulses per second to the strand and produce random transient vibrations in the strand traveling through the molten coating metal characterized by the presence of innumerable frequencies in excess of about 80 c.p.s. and an overall acceleration value in excess of 20 g, positive vibration dissipating means at the exit end of the bath adapted to contact said strand prior to its discharge into the air, adjustable means for urging the strand into contact with the vibrating means, and variable speed driving means for the vibrating means, said driving means being adapted to rotate the vibrating means so that the impact is applied in the direction of movement of the strand.

6. Apparatus for continuously hot-dip coating strand comprising means for continuously advancing strand through a bath of molten coating metal in a substantially untensioned condition, rotary vibrating means at the entry end of the bath for imparting at least 40 shock type impulses per second to the strand and produce random transient vibrations in the strand traveling through the molten coating metal characterized by the presence of innumerable frequencies in excess of about 80 c.p.s. and an overall acceleration value in excess of 20 g, positive vibration dissipating means at the exit end of the bath adapted to contact said strand prior to its discharge into the air, and driving means for the rotary vibrating means, said driving means being adapted to rotate the

**11**

rotary vibrating means so that the impact is applied in  
the direction of movement of the strand.

**References Cited in the file of this patent****12**

|              |       |                |
|--------------|-------|----------------|
| Brondyke     | ----- | Jan. 17, 1956  |
| Jones et al. | ----- | July 21, 1959  |
| Linden       | ----- | Aug. 18, 1959  |
| Baker        | ----- | Sept. 29, 1959 |

**UNITED STATES PATENTS****5**

|           |      |       |               |
|-----------|------|-------|---------------|
| 1,770,910 | Byrd | ----- | July 22, 1930 |
| 1,933,401 | Ward | ----- | Oct. 31, 1933 |